

March 12, 1929.

F. E. OWEN

1,705,094

REFRACTORY RESISTOR SUPPORTING PLATE

Filed Nov. 4, 1927



BY Wm Bieber  
ATTORNEY

## UNITED STATES PATENT OFFICE.

FREDERICK E. OWEN, OF EAST PALESTINE, OHIO.

## REFRACTORY RESISTOR-SUPPORTING PLATE.

Application filed November 4, 1927. Serial No. 231,000.

My invention relates to electric heating units and particularly to refractory resistor-supporting plates therefor.

An object of my invention is to provide a relatively simple, compact, and inexpensive resistor-supporting plate.

Another object of my invention is to provide a refractory resistor-supporting and heat-insulating plate embodied in a unitary structure.

In practicing my invention, I provide a fired refractory ceramic resistor-supporting plate of substantially standard design and construction, having closely adherent to one of its surfaces, a relatively thick layer of heat-insulating material that has been air-dried in its proper operative position relatively to the fired plate.

The desirability or necessity for providing a layer of heat-insulating material below a refractory heater brick has long been recognized and it has heretofore been customary to make the two members entirely separate from one another. This means that the relatively brittle heat-insulating plate must be manufactured and handled separately, with the result that too large a percentage thereof are chipped or broken in shipment or in assembly. The device embodying my invention provides, as noted above, a unitary assembly embodying both parts.

In the single sheet of drawings,

Figure 1 is a view, in vertical section, of a unitary heater brick embodying my invention,

Fig. 2 is a view, in vertical section, of a device embodying my invention shown during its process of manufacture,

Fig. 3 is a bottom plan view, with portions broken away, of a modified form of device embodying my invention, and

Fig. 4 is a view, in lateral section therethrough, taken on the line IV—IV of Fig. 3.

A refractory ceramic heater brick 11 is shown in vertical section in Figs. 1 and 2 of the drawings and may be of any desired size, shape, and contour. I have shown a substantially circular brick, which is provided, in one face thereof with a spiral groove 12 having walls 13 located between adjacent grooves. A helically-wound resistor wire 14 is located within the groove 12. Bridges 15 extend across the groove 12 at spaced intervals in order to retain the resistor wire 14 within the otherwise open groove 12.

Openings 16 extend through the body por-

tion of the plate 11 beneath the bridge 15, these openings being made necessary by the use of rods provided in the molds in order to permit of molding the bridges 15 at the same time that the body portion of the heater brick is being molded. The use of these rods is of course, well known in the art. This brick is molded, air-dried, and then fired in the usual manner.

A single central opening 17 is also provided to permit the inner end of the resistor wire 14 to extend downwardly through the body portion of the plate 11. The other end of the resistor wire extends downwardly through a suitable opening near the periphery of the plate, this opening not being shown in the drawing.

A relatively heavy plate or layer 18 of refractory heat-insulating material is located closely adjacent and cemented to the bottom surface of the plate 11. Integral portions of the heat-insulating plate extend a small distance into the openings 16 and are indicated at 19. The material comprising the layer 18 consists of infusorial earth or kieselguhr having semi-refractory qualities and plaster Paris, about equal quantities of each being used. The materials are mixed while dry and are then moistened with water before using.

The method of manufacture is substantially as follows:—the heater brick 11 after having been molded and fired is permitted to cool. Its upper surface is then laid on a suitable bench or other plane surface 21 and a clamping ring 22 is placed therearound fitting tightly thereon. Any suitable device may be employed effective for the purpose desired, namely to provide a peripheral wall for a plastic mass of the above mentioned heat-insulating mixture. The central opening 17 is filled with a rod 23. The openings 16 are filled with small masses 19 of the mixture of kieselguhr and plaster Paris, the consistency of which is such that an operator can place the quantities 19 in the openings 16 to close them.

The moistened mixture is then poured into the mold thus provided and is allowed to dry in the open air until thoroughly dry. I have found that a layer 18 thus made adheres closely to the adjacent surface of the heater brick by its own cementing action and is held also by the small masses 19 located within the openings in the fired heater brick.

Figs. 3 and 4 show a modified form of structure embodying my invention. A re-

refractory ceramic brick 31 of plate form embodies a groove 32 for receiving a resistor 33 therein. Bridges 34 integral with the walls 35 of the grooves are provided, all as hereinbefore set forth in connection with the device shown in Figs. 1 and 2. The brick or plate 31 embodies also an integral peripheral depending flange portion 36 and a plurality of radially-extending integral bottom ribs 37, an integral central hub portion 38 being also provided.

A mass 39 of a mixture of infusorial earth and plaster Paris, as hereinbefore described, is located in each of the sections defined by a 15 part of the depending flange 36 portion and two adjacent radial ribs 37. Small masses 41, of the same mixture, are pressed into the openings 42 under the bridges 34, all as has hereinbefore been described. The masses 39 20 of the mixture of infusorial earth and plaster Paris will adhere closely to the bottom surface of the brick 31 and to the small masses 41 by their inherent cementing action. The masses 39 are air-dried as was hereinbefore 25 described.

The amount of the mixture of infusorial earth and plaster is just sufficient to fill the recess, the bottom surface of the masses being even with the bottom edge of the flange 36 and of the ribs 37. The brick may be located in an inverted position on a suitable table or support 44 during this operation. The heat-insulating material interfits with the fired ceramic brick constituting a unitary 35 assembly in which one mass of material supports the other.

A unitary structure of this kind is relatively inexpensive and will withstand a relatively large amount of handling during shipment and assembly without serious danger of cracking or breaking off of the heat-insulating material which has been cemented against the refractory ceramic brick.

The device embodying my invention thus 45 provides a relatively simple, compact, and

effective unitary structure embodying a fired refractory ceramic resistor-supporting plate and a layer of refractory heat-insulating material located closely adjacent and adherent to one surface of the fired plate, the heat-insulating material being air-dried only.

Various modifications may be made in the device embodying my invention and I desire that only such limitations shall be placed thereon as are imposed by the prior art or are set forth in the appended claims.

I claim as my invention:

1. As a new article of manufacture of the class described, a unitary self-supporting assembly consisting of a ceramic resistor-supporting plate and a layer of heat-insulating material located against one surface only thereof opposite to its heating surface and inherently cemented thereagainst.

2. As a new article of manufacture of the class described, a unitary assembly comprising a ceramic resistor-supporting plate, and a layer of heat-insulating material comprising infusorial earth and plaster Paris inherently cemented against one surface of the refractory plate.

3. As a new article of manufacture of the class described, a unitary assembly comprising a ceramic resistor-supporting plate, having openings therethrough, and a layer of heat-insulating material located against and inherently cemented to one surface of the plate and having portions thereof extending into the openings in said plate.

4. As a new article of manufacture of the class described, a unitary assembly comprising a fired plate of refractory material and a layer of a mixture of a comminuted heat-insulating material and a binder of plaster Paris molded into intimate contact with one surface only of said plate to inherently cement said layer to said plate.

In testimony whereof, I have hereunto subscribed my name this 29 day of October, 1927.

FREDERICK E. OWEN.